

May 1, 1962

E. C. JENNINGS ET AL  
COATING COMPOSITION OF POLYVINYL ACETATE, WERNER  
COMPLEX, AND QUATERNARY AMMONIUM COMPOUND, AND  
PAPER COATED THEREWITH

3,032,523

2 Sheets-Sheet 1

Filed May 21, 1959



INVENTORS  
EDWARD C. JENNINGS  
MONROE. F. SMITH

BY *Fryer & Johnson*  
ATTORNEYS

May 1, 1962

E. C. JENNINGS ET AL  
COATING COMPOSITION OF POLYVINYL ACETATE, WERNER  
COMPLEX, AND QUATERNARY AMMONIUM COMPOUND, AND  
PAPER COATED THEREWITH

3,032,523

Filed May 21, 1959

2 Sheets-Sheet 2

FIG-3



INVENTORS  
EDWARD C. JENNINGS  
MONROE F. SMITH  
BY *Fryer & Johnson*  
ATTORNEYS

## 1

3,032,523

## COATING COMPOSITION OF POLYVINYL ACETATE, WERNER COMPLEX, AND QUATERNARY AMMONIUM COMPOUND, AND PAPER COATED THEREWITH

Edward C. Jennings, Antioch, and Monroe F. Smith, Walnut Creek, Calif., assignors to Fibreboard Paper Products Corporation, San Francisco, Calif., a corporation of Delaware

Filed May 21, 1959, Ser. No. 814,931

8 Claims. (Cl. 260—29.6)

This invention relates to water repellent coating compositions for paperboard and the like, and more particularly to an improved moisture resistant composition comprising polyvinyl acetate, a quaternary ammonium compound and a Werner type chromium complex. Such coating compositions do not adhere to each other even under humid or moist conditions. The tendency of coatings to adhere or stick to each other is known as blocking. This application is a continuation in part of application Serial No. 477,362, filed December 23, 1954, now abandoned.

Water soluble compounds of the Werner type in which trivalent nuclear chromium atoms are coordinated with carboxylic acid groups are described in United States Letters Patent No. 2,273,040, No. 2,359,958, and No. 2,544,666, and compounds of such character are referred to herein as Werner type chromium complexes or as Werner type complexes. Werner type complexes have been employed as surface coatings, both alone and as additives to various coating compositions, to provide increased water repellent characteristics. However, for some purposes, the amount of moisture resistance provided by Werner type complexes is not all that is to be desired.

One use of Werner type complexes has been as an additive to polyvinyl acetate coatings for paperboard carton blanks in order to reduce blocking of such coatings when the blanks are placed in a stack. This blocking makes it particularly difficult to separate individual blanks from stacks of such blanks by automatic feeding means which feed the blanks to carton setting up machinery. Although the Werner type chromium complex that has a carboxylic acid group of at least ten carbon atoms reduces the blocking of polyvinyl acetate coatings under warm and dry conditions, considerable blocking is obtained under humid or moist conditions when such a Werner type complex is the only moisture repellent additive incorporated in the coating. Werner type complexes with carboxylic acid groups having less than ten carbon atoms are not generally very effective moisture repellent compounds when employed alone. It would be advantageous to reduce the problem of blocking of polyvinyl acetate coatings in the presence of moisture, since the oil and fat resistant polyvinyl acetate coatings for paper products are otherwise very desirable for packaging greasy articles.

In summary, this invention comprises the provision of a polyvinyl acetate coating for paperboard or the like, which coating has increased moisture resistance due to the incorporation of a quaternary ammonium compound having a carbon chain of at least about six carbon atoms in length, together with a water soluble Werner type complex that has a trivalent nuclear chromium atom coordinated with a carboxylic acid group. Such Werner type complexes that have carboxylic acid groups of at least ten carbon atoms provide optimum water repellency characteristics in the polyvinyl acetate coating composition. However, when a quaternary ammonium compound is employed in the composition together with the Werner type

## 2

complex in accordance with this invention, the number of carbon atoms on the carboxylic acid group of the Werner type complex is not critical, since sufficient water repellency may be obtained from a long carbon chain on the 5 quaternary ammonium compound. Either the Werner type complex or the quaternary ammonium compound, or preferably both, should have a long carbon chain for optimum results.

The composition of this invention comprising polyvinyl acetate, a quaternary ammonium compound and a Werner type chromium complex is employed with particular advantage in the form of an aqueous emulsion for coating paperboard or the like. Paperboard having such coatings have much less blocking than other polyvinyl acetate 15 coatings, particularly under conditions of moisture and high humidity. Consequently, paper products having coatings of polyvinyl acetate incorporating the Werner complex and quaternary ammonium compound may be stacked and stored under humid conditions without 20 encountering a blocking problem. The composition hereof is particularly useful for coating paperboard carbon blanks, but is also useful for coating other thinner paper products. For convenience all such paper products are referred to herein as paperboard.

25 Best results are obtained when at least one mol of the quaternary ammonium compound is included in the polyvinyl acetate composition for each mol of the Werner type chromium complex. Also, quaternary ammonium compounds having at least one chain of six and preferably 30 more carbon atoms attached to the nitrogen atom are most effective in providing increased moisture resistance with the Werner type complex, and thus are employed in the composition.

The combination of a quaternary ammonium compound with a Werner type chromium complex in the polyvinyl acetate composition produces a coating having greater resistance to moisture than a like coating which includes either of such compounds alone without the presence of the other. The water resistance provided by the 35 Werner type chromium complex is attributed to the outward orientation of long chain fatty acid groups in the molecule, and it is believed that the additional water repellent effect obtained by inclusion of the quaternary ammonium compound is obtained because it masks the 40 exposed carbonyl oxygen groups of the acid in the Werner type chromium complex, and increases water repellency 45 due to its additional long carbon chain.

With reference to the drawings, FIG. 1 is a graph illustrating the decrease in blocking 50 under humid conditions of paperboard coated with compositions comprising polyvinyl acetate, quaternary ammonium compound, and a Werner type chromium complex as the number of carbon atoms in the longest carbon chain on the nitrogen atom of the quaternary ammonium compound is increased.

FIG. 2 is a graph illustrating the change in blocking force under humid conditions of paperboard coated with compositions comprising polyvinyl acetate, quaternary ammonium compound and a Werner type chromium complex as the mol ratio of quaternary ammonium compound to Werner type chromium complex in the coating composition is increased.

FIG. 3 is a graph illustrating the change in humid 65 blocking of paperboard coated with a composition comprising polyvinyl acetate, quaternary ammonium compound and a Werner type chromium complex as the proportion of Werner type complex in the coating composition is varied while the mol ratio of quaternary ammonium

nium compound to Werner type chromium complex is maintained equal to one.

In greater detail, any of the well known water soluble Werner type chromium complexes in which a trivalent nuclear chromium atom is coordinated with a substituted or unsubstituted carboxylic acid group may be employed in the polyvinyl acetate compositions of this invention. Carboxylic acid groups having at least ten carbon atoms should preferably be employed in this invention since they provide the greatest water repellent effect. However, as previously described, carboxylic acid groups having less than ten carbon atoms are suitable for use in conjunction with quaternary ammonium compounds having long carbon chains. Werner type complexes having acyclic acid groups of at least ten carbon atoms and the method of their preparation are described in United States Letters Patent No. 2,273,040, while those having cyclic acid groups are described in United States Letters Patent No. 2,359,858. Also, Werner type complexes having acid groups of less than ten carbon atoms in length are readily prepared, as is well known, in the manner described in the aforementioned patents by employing an organic acid or acid anhydride having a chain length of less than ten carbon atoms. Patent No. 2,544,666 relates to the preparation of such complexes having unsaturated acid groups. A readily available and useful Werner type complex, namely stearato chromic chloride, is sold in an isopropanol solution by E. I. du Pont de Nemours & Company under the name "Quilon." "Quilon" contains 29% to 30% by weight stearato chromic chloride, 65% to 70% by weight isopropanol, and less than 5% water.

An example of a suitable Werner type complex having a carboxylic acid group of less than ten carbon atoms in length is methacrylato chromic chloride sold by E. I. du Pont de Nemours & Co. in an isopropanol solution under the name "Volan." This compound has a straight chain length of three carbon atoms attached to the carboxylic acid group of the Werner type complex.

Any quaternary ammonium compound may be employed together with the Werner type complex in accordance with this invention to obtain increased moisture resistance and reduction of blocking of coatings. It is the quaternary ammonium nitrogen which is the essential element in the composition, and the character of the four organic radicals is of no importance or significance in obtaining the desired low blocking polyvinyl acetate coating composition except that at least one of the organic radicals must contain a straight carbon chain at least six carbon atoms in length. Likewise, the nature of the anion on the quaternary ammonium compound is of no importance since the anion plays no part or function in providing the low blocking properties, and thus any anion may be present on the quaternary ammonium compound.

The term quaternary ammonium compound as used herein has well defined meaning, and it is given in Webster's New International Dictionary, 2nd edition, as "a base or salt which may be regarded as a compound of ammonium in which all four hydrogen atoms are replaced by organic radicals." More particularly in chemical terms, such compounds may be designated by the formula:  $(R_4N)^+X^-$  in which the R's are any suitable organic radical, N is nitrogen, and X is any anion. Each of the R groups may be any saturated or unsaturated, unsubstituted or substituted, alkyl or aryl groups, acyclic radicals, cyclic radicals of carbon atoms, cyclic radicals containing nitrogen in the ring such as isoquinolinium, aryl-alkyl combinations in one chain, and radicals containing ether linkages. Even alkyl pyridinium compounds may be used as the quaternary ammonium compound. As mentioned above, at least one of the R groups attached to the nitrogen atom should contain an alkyl or alkylene group having at least one straight chain of approximately six or more carbon atoms, although all of

the R groups may be long chain groups. However, more than one long chain of carbon atoms attached to the nitrogen atom produces no additional water repellent effect. Although the alkylol-alkyl derivatives and the alkyl-isoquinolinium derivatives of the quaternary ammonium compounds provide low blocking values even under moist conditions when employed with the described Werner type complexes, they have certain properties, such as poor wetting or mottle, which render them less desirable as additives than the quaternary ammonium compounds having alkyl or alkylene groups. Examples of specific quaternary ammonium compounds that may be employed are given in Table I, explained more fully hereinafter, it being understood that of the quaternary ammonium compounds listed therein, those having hydrocarbon chains attached to the nitrogen atom are preferred. Examples of anions X which may be in the quaternary ammonium compound include sulfate, nitrate, iodide, hydroxyl, formate, acetate, phosphate, polyacrylate, alginic, bromide, and chloride. The chlorides are preferred because of their ready availability.

Quaternary ammonium compounds that are either soluble or insoluble in aqueous media are useful for the purposes of this invention. When the quaternary ammonium compound is employed in a coating composition for paperboard which is to contain food products, it is generally desirable to use a water insoluble quaternary ammonium compound in order to insure against the possibility of extraction of the quaternary ammonium compound from the coating into the food.

Water insoluble quaternary ammonium compounds may be prepared from soluble quaternary ammonium compounds either prior to addition of the compound to the coating composition, or in situ after the soluble quaternary ammonium compound has been incorporated in the liquid coating composition. Such insoluble quaternary ammonium compounds are readily prepared by reacting soluble quaternary ammonium compounds with a high molecular weight acid or preferably a polymeric polyacid, such as polyacrylic acid, carboxymethyl cellulose, or polyanhydro-beta-d mannuronic acid, alginic acid, or with the alkali metal and ammonium salts of such acids. Such polymeric polyacids are well known and they are characterized by the following repeating group in which n is at least 2 and is preferably large enough to render the quaternary ammonium compound insoluble. Such polymeric polyacids may also be called synthetic resinous polymers having a plurality of organic acid groups:



The H is hydrogen, C is carbon, and O is oxygen. Hydrogen may be replaced by a cation such as sodium, potassium or ammonium. Regardless of what cation is present, the polymeric polyacid is readily reacted with a quaternary ammonium compound by replacement of the cation with the quaternary radical to form the insoluble quaternary ammonium compound.

Furthermore, it is known that the soluble betaine derivatives of quaternary ammonium salts are nontoxic, and that such betaine derivatives are natural components of many food-stuffs. Since the betaine derivatives of quaternary ammonium salts also provide resistance to moisture and reduction of humid blocking in accordance with this invention, they may likewise be advantageously employed in coating compositions for paperboard containers used for food products. Betaine derivatives of quaternary ammonium salts are substituted or unsubstituted quaternary ammonium betaines which are inner salts having the formula  $(R_1R_2R_3N)^+(CH_2COO)^-$  wherein R<sub>1</sub>, R<sub>2</sub> and R<sub>3</sub> represent any organic radical. Examples of suitable betaine derivatives are cholesteryl, cetyl and melissyl

betaine, quaternary ammonium salts. Another specific example of a water soluble betaine quaternary ammonium compound which may be employed as the quaternary ammonium compound is betaine trimethylglycocol which has the following structural formula:



The polyvinyl acetate composition is most conveniently applied as a protective coating for paperboard in the form of an aqueous emulsion. The incorporation of a quaternary ammonium compound, and Werner type complex in polyvinyl acetate emulsions provides a coating having very low blocking. Polyvinyl acetate emulsions are sold by E. I. du Pont de Nemours & Company under the trademark "Elvacet." The "Elvacet" compositions contain about 55% by weight of resin solids, and are sold in varying viscosities depending upon the degree of polymerization desired. Such polyvinyl acetate coatings exhibit considerable blocking under humid conditions, even when a Werner type complex having a carboxylic acid group of at least ten carbon atoms is included alone as the water repellent additive in the coating. The incorporation of a quaternary ammonium compound in such polyvinyl acetate coating compositions along with the Werner type complex produces marked results in reducing the humid blocking of such coatings. Polyvinyl alcohol is generally present in such coatings, and the composition of this invention likewise has a marked effect in rendering this compound moisture resistant.

Although plasticizers for the polyvinyl acetate need not be present in the composition, it is usually desirable to include any of the well known suitable plasticizers in order to increase flexibility of the coating. Examples of suitable plasticizers are butyl phthalyl butyl glycolate and methyl phthalyl ethyl glycolate.

Also, for many purposes it is desirable to include a pigment in the composition to mask the characteristic green color of the Werner type complex in which trivalent chromium is co-ordinated with carboxylic acid groups. Examples of compounds that may be employed for this purpose are titanium dioxide, zinc sulfide, and talc. Titanium dioxide is preferred because of its effectiveness in masking the green color. If the color of the Werner type complex is unobjectionable for the purposes for which the composition is to be employed, the pigment may be omitted.

The addition of even a very small amount of quaternary ammonium compound to the Werner type complex provides improved water repellent characteristics. A mol ratio of quaternary ammonium compound to Werner type complex of as little as 0.1 results in much greater water repellent characteristics than is obtained with the Werner type complex alone. As the ratio of quaternary ammonium compound to Werner type complex is increased to about 0.25, rapid improvement in moisture resistance is obtained. With further increases in the proportion of quaternary ammonium compound until a mol ratio of 1.0 the improvement in moisture resistance is more gradual. Increasing the proportional amount of quaternary ammonium compound to Werner type complex to mol ratios greater than 1.0 provides little additional improvement. Consequently, a mol ratio of about 1.0 is preferred for best results. A maximum mol ratio of quaternary ammonium compound to Werner type complex of 50 should not be exceeded as quaternary in excess of a one to one mol ratio contributes nothing, and above 50 to one excessive dilution by the quaternary is obtained.

When the quaternary ammonium compound and Werner type complex is employed to lower the blocking of polyvinyl acetate coating compositions, any amount of Werner type complex will reduce blocking as shown in Table III, explained more fully hereinafter. Generally, it is advisable to employ at least about 0.1% by weight Werner type complex based on the weight of polyvinyl acetate resin solids. A rapid reduction of humid blocking is obtained as the amount of Werner type complex is increased to about 0.5% or more by weight, based on the weight of the polyvinyl acetate resin solids. Further increases in the amount of Werner type complex until about 2% by weight is reached provides a less rapid reduction in humid blocking, and increasing the amount of Werner type complex above 2% by weight provides little advantage. The greater the amount of Werner type complex employed, the more intense the green color becomes and the more difficulty is encountered in masking the color.

If a plasticizer is included in the coating composition, the amount of plasticizer employed depends upon the degree of flexibility desired in the coating. If a relatively stiff coating is suitable, very little plasticizer is needed and the plasticizer may even be omitted. More than 10% by weight plasticizer based on the total weight of non-volatile constituents in the coating tends to unduly increase the blocking characteristics of the coating. Polyvinyl acetate coating compositions for paperboard carton blanks preferably employ between 2% to 7% by weight plasticizer based on the total weight of such non-volatile constituents.

As previously described, it is not necessary to include a pigment in the composition. However, sufficient pigment is employed in the coating composition of polyvinyl acetate, quaternary ammonium compound, Werner type complex and plasticizer to mask the green color of the Werner type complex if the color is objectionable. No pigment is necessary if the green color is unimportant. From 5% to 15% by weight pigment based on the weight of non-volatile constituents in the coating composition is usually preferred. Below 5% by weight of pigment may not be sufficient to mask the green color, and in coatings for paperboard employed for food products, it is usually desirable that the color be masked. If more than about 40% by weight pigment is employed, the coatings tend to become unduly stiff.

The range of proportions of the three essential ingredients in the coating composition which form the solid coating are as follows in terms of solids present on the dry basis:

|                              | Percent by weight |
|------------------------------|-------------------|
| Polyvinyl acetate            | 85 to 99.85       |
| Werner type chromium complex | 0.1 to 14.95      |
| Quaternary ammonium compound | 0.05 to 14.9      |

The following composition range summarizes the preferred amounts of the components employed in a commercial paperboard coating for paperboard carton blanks. However, the ingredients other than the polyvinyl acetate, Werner complex and quaternary ammonium compound are not essential, as previously described. All weights herein are given on the basis of the actual weight of the specified compound, not including the weight of water or alcohol or other volatile solvent present in the liquid emulsion mixture.

|                                                                                | Percent by weight |
|--------------------------------------------------------------------------------|-------------------|
| Polyvinyl acetate                                                              | 59 to 91.65       |
| Werner type chromium complex                                                   | 0.25 to 10        |
| Quaternary ammonium compound                                                   | 0.1 to 5          |
| Pigment                                                                        | 5 to 15           |
| Suspending agent (any conventional suspending agent such as polyvinyl alcohol) | 0.5 to 4          |
| Plasticizer                                                                    | 2 to 7            |

It is apparent that the coating is composed of a major

proportion of polyvinyl acetate and minor proportions of the remaining components. As previously explained, a satisfactory coating may be prepared with very little Werner type complex and quaternary ammonium compound. Also, the pigment suspending agent and plasticizer may be omitted. Furthermore, an amount of the complex and the quaternary ammonium compound considerably in excess of the range indicated may be employed in preparation of suitable coatings although no appreciable improvement in resistance to moisture is obtained by such procedure. The optimum amount of quaternary ammonium compound to employ is best determined in terms of the mol ratio of quaternary ammonium compound to Werner type chromium complex, since the molecular weight of the quaternary ammonium compound may vary considerably.

The composition comprising polyvinyl acetate, the Werner type complex and the quaternary ammonium compound may be prepared by simply mixing the compounds in water to form an emulsion. The Werner type complex of the character described herein is readily soluble in water. Also, most quaternary ammonium compounds are soluble in water. If a water insoluble quaternary ammonium salt is employed, it may be incorporated in the composition as a dispersion. However, it is usually more convenient to insolubilize a soluble quaternary ammonium compound in situ by adding a polymeric polyacid after the soluble ammonium compound has been mixed with the Werner type complex. Best results are obtained when the composition is permitted to stand for a short period before application so that equilibrium will be reached.

The preparation of a coating composition of polyvinyl acetate having low blocking in accordance with this invention does not present any particular problem. Best results are obtained by first mixing a plasticizer, if any is used, in an aqueous emulsion of polyvinyl acetate to render the final coating flexible. Pigment for masking the green color of the Werner type complex is then preferably added in the form of a water dispersion of the pigment in polyvinyl alcohol, although the pigment may be omitted. A suspension of 20% by weight pigment, 5% by weight polyvinyl alcohol and 75% water is convenient for this purpose. Next, the Werner type chromium complex, which is conveniently dissolved in isopropanol, is incorporated by intermixing it together with the mixture of polyvinyl acetate emulsion composition. Finally, the quaternary ammonium compound is mixed into the composition. If it is desired to insolubilize the quaternary ammonium compound, this may be accomplished by adding a polymeric polyacid to the emulsion as previously explained. A short period of standing before application, such as one or two hours, provides best results since it permits the components to reach equilibrium.

Water is always included in the liquid compositions of polyvinyl acetate, Werner complex and quaternary ammonium compound so that the compositions may be applied as liquid emulsions. The water is a volatile component which evaporates to leave the remaining solids as a coating when the composition is applied to paperboard or the like. The water is present in the composition in an amount sufficient to render the composition liquid and readily applied by conventional paperboard coating methods. Regardless of whether the pigment or plasticizer are included in the coating, the amount of water employed based on the total weight of the liquid composition is between about 25% and 80% by weight water to between about 20% and 75% by weight of solids in the aqueous emulsion. If more than about 80% water is employed, the final coating becomes too thin. On the other hand if less than about 25% water is included in the liquid emulsion hereof, the composition is too viscous to apply and form a satisfactory coating.

The resultant somewhat viscous liquid coating com-

position may be applied to paperboard by any conventional coating means such as by the kiss roll method, in which the coating is applied by rollers. Although it is not necessary to heat the coating in order to cure it, best results are obtained when the coated paperboard is dried by passing it through a heated drying tunnel, or when the coating is dried by infra red rays. If no drying means is employed, an unduly long period elapses before the coating is dry enough to permit use or stacking of the paperboard. The liquid composition is applied to paperboard in an amount sufficient to provide a continuous coating when the water evaporates. Approximately 6 to 8 pounds of the liquid coating composition is preferred to provide a continuous coating for one side of 1000 square feet of paperboard, but a range of between one and 20 pounds may be utilized. This means that at least about 3 to 4 pounds of the dried coating composition is preferred for providing a water resistant coating on paperboard, but a paper product having a dry coating of between about 0.5 and 10 pounds of the composition per 1000 square feet of the product is satisfactory.

The data set forth in all of the following tables were obtained from tests employing bleached kraft paperboard coated with the coating compositions specified. The test for blocking under humid conditions was conducted by stacking specimens of the coated paperboard under a weight so that 4 square inches (2 in. x 2 in.) of the paperboard was subjected to a pressure of 4.2 pounds per square inch. The samples were exposed to a temperature of 73° F. at from 90% to 95% relative humidity for 24 hours. The blocked samples were then conditioned for 4 hours at 73° F. and 50% relative humidity while remaining under the same pressure of 4.2 pounds per square inch. The force in grams required to pull the samples apart was then measured at least ten times for each type of coating. The average force is given in the tables as the average humid blocking force.

The coating compositions tested in the following tables were prepared by mixing a polyvinyl acetate emulsion sold by E. I. du Pont de Nemours & Company under the name "Elvacet 81-900" with butyl phthalyl butyl glycolate as a plasticizer. A water dispersion of titanium dioxide suspended in polyvinyl alcohol was then mixed into the composition. The polyvinyl alcohol used was "Elvanol 54-22" sold by E. I. du Pont de Nemours & Company. Next, the Werner type chromium complex was added to the mixture, and finally the quaternary ammonium compound was mixed into the composition. The Werner type complex employed in the tests was the chromium-stearic acid complex sold by E. I. du Pont de Nemours & Company under the name "Quilon," which complex is sold in an isopropanol solution as previously explained. The total weight of water in the compositions was 50% by weight.

In Table I, the coating compositions tested contained the following components which were all the same, except that the quaternary ammonium compound was varied to determine the effects of varying the carbon chain length of one of the R groups thereof.

|                                                   | Percent by Weight of Non-volatile Constituents (not including the weight of the quaternary ammonium compound) |
|---------------------------------------------------|---------------------------------------------------------------------------------------------------------------|
| 65                                                |                                                                                                               |
| Polyvinyl acetate ("Elvacet 81-900").             | 81.0 (Resin solids in the emulsion).                                                                          |
| Plasticizer (Butyl phthalyl butyl glycolate).     | 5.8.                                                                                                          |
| 70 Pigment (titanium dioxide).                    | 8.8.                                                                                                          |
| Suspending agent for pigment (Polyvinyl alcohol). | 2.2 (Weight of resin solids).                                                                                 |
| Werner type chromium complex ("Quilon").          | 2.2 (Weight of actual complex in the solution).                                                               |
| Quaternary ammonium compound (Listed in Table I). | One mole per mole of Werner type complex.                                                                     |

9  
Table I

| Compound No. | Quaternary Ammonium Compound                                                           | Number of Carbon Atoms in Longest "R" Chain | Average Humid Blocking Force in Grams |
|--------------|----------------------------------------------------------------------------------------|---------------------------------------------|---------------------------------------|
| 0.....       | Control test with no quaternary ammonium compound employed in the composition.         | -----                                       | 360                                   |
| 1.....       | Tetraethyl ammonium bromide.                                                           | 1                                           | 271                                   |
| 2.....       | Tetraethyl ammonium bromide.                                                           | 2                                           | 248                                   |
| 3.....       | Phenyltrimethyl ammonium iodide.                                                       | 1                                           | 171                                   |
| 4.....       | Tetra (ethanol) ammonium chloride.                                                     | 2                                           | 167                                   |
| 5.....       | Tetra-n-propyl ammonium bromide.                                                       | 3                                           | 143                                   |
| 6.....       | n-tetrabutyl ammonium iodide.                                                          | 4                                           | 106                                   |
| 7.....       | (C <sub>8</sub> -C <sub>18</sub> alkyl) trimethyl ammonium chloride.                   | 13 Av.                                      | 15<br>22                              |
| 8.....       | (C <sub>12</sub> alkyl) trimethyl ammonium chloride.                                   | 12                                          | 33                                    |
| 9.....       | (C <sub>8</sub> -C <sub>18</sub> alkyl) dimethyl benzyl ammonium chloride.             | 13 Av.                                      | 34<br>4.00                            |
| 10.....      | (C <sub>16</sub> alkyl) trimethyl ammonium chloride.                                   | 16                                          | 41<br>20                              |
| 11.....      | (C <sub>16</sub> alkyl) dimethyl ethyl ammonium bromide.                               | 16                                          | 29                                    |
| 12.....      | (C <sub>18</sub> alkyl) trimethyl ammonium chloride.                                   | 18                                          | 34                                    |
| 13.....      | Di-(C <sub>8</sub> -C <sub>18</sub> alkyl) dimethyl ammonium chloride.                 | 13 Av.                                      | 32                                    |
| 14.....      | Tris (ethanol) (C <sub>12</sub> alkyl) ammonium chloride.                              | 12                                          | 4<br>25                               |
| 15.....      | Tris (ethanol) (C <sub>18</sub> alkyl) ammonium chloride.                              | 18                                          | 3<br>2                                |
| 16.....      | do                                                                                     | 18                                          | 14                                    |
| 17.....      | Tris (ethanol) (C <sub>22</sub> alkyl) ammonium chloride.                              | 22                                          | 46                                    |
| 18.....      | (C <sub>8</sub> -C <sub>18</sub> alkyl) dimethyl 3,4-dichlorobenzyl ammonium chloride. | 13 Av.                                      | 37                                    |
| 19.....      | (C <sub>12</sub> alkyl) isoquinolinium bromide.                                        | 12                                          | 2.5                                   |
| 20.....      | (C <sub>16</sub> -C <sub>20</sub> alkylene) dimethyl ethyl ammonium bromide.           | 18 Av.                                      | 16                                    |
| 21.....      | (C <sub>12</sub> alkylaryl) trimethyl ammonium chloride.                               | 12                                          | 1.6                                   |
| 22.....      | (C <sub>22</sub> alkyl) trimethyl ammonium chloride.                                   | 22                                          | 11                                    |
| 23.....      | Di-(C <sub>18</sub> alkyl) dimethyl ammonium chloride.                                 | 18                                          | 44                                    |

The data in Table I is plotted in the form of a graph in FIG. 1. In FIG. 1 the various quaternary ammonium compounds are indicated by the Compound No. assigned in Table I. The results of these tests indicate the decrease in blocking obtained with quaternary ammonium compounds as the carbon chain length of one of the organic groups attached to nitrogen in the quaternary ammonium compound is increased. It is apparent that no significant reduction in blocking occurs with quaternary ammonium compounds having attached carbon chains of a length greater than approximately six carbon atoms. The difference between the blocking of the control coating which employed a Werner type complex without the presence of a quaternary ammonium compound, and the coatings in which a quaternary ammonium compound was incorporated in the coating, indicates the importance of employing a quaternary ammonium compound in accordance with this invention. It is apparent that the quaternary ammonium compounds having at least one chain of approximately six or more carbon atoms attached to the nitrogen atom are most effective in providing increased moisture resistance.

The data in Table II illustrates the effect of increasing the mol ratio of quaternary ammonium compound to Werner type chromium complex in the coating composition. The coating compositions employed were identical to the compositions of Table I with respect to the amount and type of polyvinyl acetate, plasticizer, pigment, suspending agent and Werner type chromium complex. However, the type and amount of quaternary ammonium compound employed in the composition were varied in order to ascertain the reduction in blocking obtained with various amounts of quaternary ammonium compound. Each of the following quaternary ammonium compounds, (C<sub>8</sub>-C<sub>18</sub> alkyl) trimethyl ammonium chloride,

(C<sub>16</sub> alkyl) trimethyl ammonium chloride, (C<sub>16</sub> alkyl) dimethyl ethyl ammonium bromide, and di-(C<sub>8</sub>-C<sub>18</sub> alkyl) dimethyl ammonium chloride was employed in a coating at the mol ratios indicated in Table II in order to ascertain the reduction in blocking obtained with various amounts of quaternary ammonium compound. The blocking at each mol ratio with each quaternary ammonium compound was averaged to provide the result in the table.

Table II

| Mol Ratio of Quaternary Ammonium Compound/ Werner Type Chromium Complex | Average Humid Blocking Force in Grams |
|-------------------------------------------------------------------------|---------------------------------------|
| 0                                                                       | 360                                   |
| 0.25                                                                    | 47                                    |
| 0.50                                                                    | 39                                    |
| 1.00                                                                    | 31                                    |
| 2.00                                                                    | 27                                    |
| 4.00                                                                    | 33                                    |

Table II and the graph of the data in the table plotted in FIG. 2 illustrate that even a small amount of quaternary ammonium compound incorporated in the coating results in a marked reduction of humid blocking. It is apparent that no significant improvement is obtained by increasing the amount of quaternary ammonium in the coating composition after a mol ratio of 1.0 is obtained.

Table III lists the variation in humid blocking of polyvinyl acetate coating compositions obtained when the amount of Werner type complex in the polyvinyl acetate coating composition is varied while at the same time sufficient quaternary ammonium compound is maintained in the composition to provide a mol ratio of quaternary ammonium compound to Werner type chromium complex equal to one. The composition of the polyvinyl acetate coating is the same as that employed in Table I except that the amount of Werner type complex and quaternary ammonium compound was varied as indicated. "Quilon" was again employed as the Werner type complex, and the quaternary ammonium compound employed in the coating compositions was (C<sub>16</sub> alkyl) trimethyl ammonium chloride which is sold by Armour and Company under the name Arquad 16. The data in Table III is plotted in the form of graph in FIG. III. It is apparent that the greatest reduction in blocking occurs when about 2% by weight Werner type complex is present in the coating composition based upon the weight of polyvinyl acetate resin solids, and that no appreciable further reduction is obtained by additional increases in the amount of Werner type complex.

Table III

| Percent by weight Werner type Complex based on the Weight of polyvinyl acetate resin solids in the composition | Percent by weight Quaternary Ammonium Compound | Average Humid Blocking force in Grams |
|----------------------------------------------------------------------------------------------------------------|------------------------------------------------|---------------------------------------|
| 0                                                                                                              | 0                                              | 1,200                                 |
| 0.36                                                                                                           | 0.36                                           | 86                                    |
| 0.71                                                                                                           | 0.71                                           | 85                                    |
| 1.42                                                                                                           | 1.42                                           | 44                                    |
| 2.84                                                                                                           | 2.84                                           | 34                                    |
| 5.68                                                                                                           | 5.68                                           | 19                                    |

The following is a typical specific example of a suitable moisture resistant composition prepared in accordance with this invention. 100 parts by weight of polyvinyl acetate resin dispersion, "Elvacet Emulsion 81-900," a polyvinyl acetate emulsion sold by E. I. du Pont de Nemours & Company, and which contains approximately 55 parts by weight resin and 45 parts by weight water, was mixed with a plasticizer comprising 4 parts by weight butyl phthalyl butyl glycolate. Next 30 parts by weight of a suspension comprising 20 parts by weight titanium dioxide, 5 parts polyvinyl alcohol as a suspending agent, and 75 parts water was then added to the polyvinyl

acetate emulsion mixture. Next 5 parts by weight "Quilon," a solution of a Werner type complex sold by E. I. du Pont de Nemours & Company comprising 30 parts by weight stearato chromic chloride Werner type complex, 65 to 70 parts by weight isopropanol, and less than 5 parts by weight water was incorporated into the polyvinyl acetate coating composition with continued stirring. Finally 1½ parts by weight of a solution of 50 parts by weight of (C<sub>8</sub>-C<sub>18</sub> alkyl) trimethyl ammonium chloride in 50 parts isopropanol, a quaternary ammonium compound solution which is sold by Armour and Company under the name Arquad C, was intermixed with the composition to form the emulsion to be applied to the paperboard.

The mixture was then applied to the usual paperboard employed for making carton blanks by the conventional roll coating technique. About 8 pounds of the liquid coating composition was used in coating one side of 1000 square feet of paperboard, with 16 pounds being used for both sides.

The paperboard was then dried by passing through a drying tunnel maintained at about 120° C., with a residence time in the drying tunnel of about one minute.

Coated blanks were then cut from the rolls of coated paperboard and the blanks were then stacked and stored for two weeks under humid conditions. Very little blocking was obtained with the blanks, and they were readily separated from each other by automatic blank feeding means associated with a conventional carton setting up machine.

We claim:

1. A liquid coating composition for application to a paper product to provide a solid protective coating therefor that exhibits low blocking under both humid and dry conditions, which liquid coating composition contains water as a volatile component present in an amount to render said composition liquid, and contains as the film forming components in the solid coating in percent by weight based on the weight of said film forming components a mixture of organic compounds which consists essentially of (1) from about 85 to 99.85 percent polyvinyl acetate dispersed in said water, (2) from about 0.1 to 14.95 percent of a water soluble Werner-type chromium complex in which a trivalent nuclear chromium atom is coordinated with a carboxylic acid group, said carboxylic acid group having at least three carbon atoms, and (3) from about 0.05 to 14.9 percent by weight of a quaternary ammonium compound, said quaternary ammonium compound being selected from the group consisting of quaternary ammonium salts and quaternary ammonium bases and being present in an amount to provide a molar ratio of quaternary ammonium compound divided by said Werner-type chromium complex of at least 0.1 and not in excess of 50, and said quaternary ammonium compound having a straight carbon chain of at least six consecutive carbon atoms attached to the nitrogen atom of said compound, said coating composition containing plasticizer for said polyvinyl acetate present in an amount less than 10 percent by weight of non-volatile constituents in said coating composition.

2. The liquid coating composition of claim 1 in which said quaternary ammonium compound is water insoluble.

3. A liquid coating composition for application to a paper product to provide a solid protective coating therefor that exhibits low blocking under both humid and dry conditions, which liquid coating composition contains between about 25 percent and 80 percent by weight water and between about 20 percent and 75 percent by weight solids, and contains as the film forming components in the solid coating in percent by weight based on the weight of said film forming components a mixture of organic compounds which consist essentially of (1) from about 85 to 99.85 percent polyvinyl acetate dispersed in said water, (2) from about 0.1 to 14.95 percent of a water soluble Werner-type chromium complex in which a triva-

lent nuclear chromium atom is coordinated with a carboxylic acid group, and (3) from about 0.05 to 14.9 percent by weight of a quaternary ammonium compound, said quaternary ammonium compound being selected from the group consisting of quaternary ammonium salts and quaternary ammonium bases and being present in an amount to provide a molar ratio of quaternary ammonium compound divided by said Werner-type chromium complex of at least 0.1 and not in excess of 50, said quaternary ammonium compound having a straight carbon chain of at least six consecutive carbon atoms attached to the nitrogen atom of said compound, and said carboxylic acid group on said Werner-type chromium complex having at least ten carbon atoms, said coating composition containing plasticizer for said polyvinyl acetate present in an amount less than 10 percent by weight of non-volatile constituents in said coating composition.

4. A liquid coating composition for application to a paper product to provide a solid protective coating therefor that exhibits low blocking under both humid and dry conditions, which liquid coating composition consists essentially of water as a volatile component present in an amount to render said composition liquid, and as components which form the solid coating based on the weight of such components in said composition, from 59 to 91.65 percent by weight polyvinyl acetate dispersed in said water, from 0.25 to 10 percent by weight of a water soluble Werner-type chromium complex in which a trivalent nuclear chromium atom is coordinated with a carboxylic acid group, from 0.1 to 5 percent by weight of a quaternary ammonium compound, from 5 to 15 percent by weight of a pigment, from 2 to 7 percent by weight of a plasticizer for said polyvinyl acetate, and from 0.5 to 4 percent suspending agent for said pigment, said quaternary ammonium compound being selected from the group consisting of quaternary ammonium salts and quaternary ammonium bases and being present in an amount to provide a molar ratio of quaternary ammonium compound divided by said Werner-type chromium complex of at least 0.1 and not in excess of 50, said quaternary ammonium compound having an aliphatic hydrocarbon group containing a straight carbon chain of at least six consecutive carbon atoms attached to the nitrogen atom of said compound, and said carboxylic acid group on said Werner-type chromium complex having at least ten carbon atoms.

5. The liquid coating composition of claim 4 in which the amount of water in said composition is between 25 percent and 80 percent by weight of the composition, and the solids that form said coating comprise between about 20 percent and 75 percent of the weight of said coating composition.

6. A paper product having a solid protective coating thereon that exhibits low blocking values under both humid and dry conditions, which solid coating contains as film forming components in the solid coating a mixture of organic compounds which consists essentially of (1) from about 85 to 99.85 percent polyvinyl acetate, (2) from about 0.1 to 14.95 percent of a water soluble Werner-type chromium complex in which a trivalent nuclear chromium atom is coordinated with a carboxylic acid group, said carboxylic acid group having at least three carbon atoms, and (3) from about 0.05 to 14.9 percent of a quaternary ammonium compound, said quaternary ammonium compound being selected from the group consisting of quaternary ammonium salts and quaternary ammonium bases and being present in an amount to provide a molar ratio of quaternary ammonium compound divided by said Werner-type chromium complex of at least 0.1 and not in excess of 50, and said quaternary ammonium compound having an aliphatic hydrocarbon radical containing a straight carbon chain of at least six consecutive carbon atoms attached to the nitrogen atom of said salt, said coating containing plasticizer for said

polyvinyl acetate present in an amount less than 10 percent by weight of solids in said coating.

7. The paper product of claim 6 in which said carboxylic acid group on said Werner type chromium complex has at least ten carbon atoms.

8. A paper product having a solid protective coating thereon that exhibits low blocking values under both humid and dry conditions, which solid coating consists essentially from 59 to 91.65 percent by weight polyvinyl acetate, from 0.25 to 10 percent by weight of a water soluble Werner-type chromium complex in which a trivalent nuclear chromium atom is coordinated with a carboxylic acid group, from 0.1 to 5 percent by weight of a quaternary ammonium compound, from 5 to 15 percent by weight of a pigment, from 2 to 7 percent by weight of a plasticizer for said polyvinyl acetate, and from 0.5 to 4 percent suspending agent for said pigment, said quaternary ammonium compound being selected from the group consisting of quaternary ammonium salts and quaternary

ammonium bases and being present in an amount to provide a molar ratio of quaternary ammonium compound divided by said Werner-type chromium complex of at least 0.1 and not in excess of 50, said quaternary ammonium compound having an aliphatic hydrocarbon group containing a straight carbon chain of at least six consecutive carbon atoms attached to the nitrogen atom of said compound, and said carboxylic acid group on said Werner-type chromium complex having at least ten carbon atoms.

References Cited in the file of this patent

UNITED STATES PATENTS

|    |           |                     |               |
|----|-----------|---------------------|---------------|
| 15 | 2,346,755 | Hemming -----       | Apr. 18, 1944 |
|    | 2,673,824 | Biefeld -----       | Mar. 30, 1954 |
|    | 2,733,182 | Dalton et al. ----- | Jan. 31, 1956 |
|    | 2,801,189 | Collier -----       | July 30, 1957 |